

# UNITED STATES PATENT OFFICE.

LAWRENCE E. BARRINGER, OF SCHENECTADY, NEW YORK, ASSIGNOR TO GENERAL ELECTRIC COMPANY, A CORPORATION OF NEW YORK.

## MOLDED RESISTANCE.

No. 902,048.

Specification of Letters Patent.

Patented Oct. 27, 1908.

Application filed February 2, 1906. Serial No. 299,143.

*To all whom it may concern:*

Be it known that I, LAWRENCE E. BARRINGER, a citizen of the United States, residing at Schenectady, in the county of Schenectady, State of New York, have invented certain new and useful Improvements in Molded Resistances, of which the following is a specification.

This invention relates to resistance conductors for electric circuits and has for its object the provision of a device of this character, the resistance of which may be varied within a considerable range by varying the composition and which at the same time will 10 withstand a high temperature without injury, in addition to having sufficient strength for general use and being exceedingly cheap, efficient and durable.

My invention relates more specifically to 20 what is known in the art as molded resistance sticks. This type of resistance has been well-known for some time but has never been a success practically, because of certain objections which it has been found difficult to 25 overcome.

It is the object of my invention to overcome so far as possible the objections heretofore urged against this type of resistance.

In many of the types heretofore suggested 30 a high temperature is essential to the hardening of the compound. In others the compound air dries. The air-dried compounds require considerable time and do not produce the hard, dense, refractory substance which 35 is required for general utility in electrical work, while the fired or baked compounds are difficult to make uniformly because of oxidation of the conducting material during baking or inequalities in shrinkage, producing 40 varying resistance.

I have found that by mixing a conducting material with substances which may be treated so as to produce a silicate an exceedingly efficient resistance stick may be produced. In carrying out my invention, therefore, I mix the desired quantity of the conducting substance, which may be graphite, magnetite, carborundum, or any similar conducting material in powdered or comminuted 45 form, with suitable quantities of calcium or magnesium hydrate and silica, or flint. The quantity of conducting material will of course vary with the resistance required and the amounts of the other materials may also

be varied within a considerable range, dependent upon the use to which the resistance is to be subjected. The percentage of conducting material may be as high as 70% or 80%, while a suitable proportion of calcium hydrate to flint in the composition of the binding base may be approximately 2 to 3. After the materials are thoroughly mixed, the mixture is compressed to produce a dense mass. This mass is then subjected to steam treatment, the pressure of which, and, therefore, the temperature, will depend somewhat upon the proportions of materials used and also upon the time which is to be consumed in hardening. A pressure of 150 lbs., corresponding to a temperature of 181° C., has been found to be sufficient to harden certain compositions in about five hours. The steam converts the calcium hydrate and silica into a hydrous silicate of calcium, which makes a strong binder for the conducting material. As a substitute for calcium hydrate, I have found that powdered magnesium hydrate or magnesium oxid may be used.

It will be seen that I have produced a resistance stick having properties which render it valuable for use under a variety of conditions. It is exceedingly hard and strong and will stand a high temperature without injury. Many modifications of my invention will suggest themselves to those skilled in the art, and it should be understood that I do not limit my invention to the combination of materials or the process of forming and arranging same herein mentioned, but that all such modifications will come within the spirit of my invention in so far as they fall within the scope of the claims annexed to and forming part of this specification.

What I claim as new and desire to secure by Letters Patent of the United States, is:

1. A resistance conductor comprising a steam-hardened compound of a conducting material and a hydrated non-conducting material.
2. A resistance conductor comprising a steam-hardened compound of a comminuted conducting material with silica and a hydrate.
3. A resistance conductor comprising a compound of a comminuted conducting material and a hydrous silicate.
4. A resistance conductor comprising a

steam-hardened compound of a comminuted conducting material with silica and calcium hydrate.

5. A resistance conductor comprising a compound of a comminuted conducting material and hydrous silicate of calcium.

6. The process of making resistance conductors which consists in mixing a comminuted conducting material with suitable 10 quantities of silica and a hydrate and subsequently treating the mixture to produce a hydrous silicate.

7. The process of making resistance conductors which consists in mixing a comminuted conducting material with suitable 15 quantities of silica and a hydrate and subsequently treating the mixture with steam to harden the same.

8. The process of making resistance sticks 20 which consists in mixing a comminuted con-

ducting material with definite quantities of calcium hydrate and silica, compressing the mixture to produce a dense mass, and subsequently treating the mass with steam to harden the same.

9. The process of making resistance conductors which consists in mixing a comminuted conducting material with suitable quantities of silica and any base which will combine with it to form a hydrous silicate 30 under the influence of steam treatment, and subsequently treating the mixture to produce a hydrous silicate.

In witness whereof, I have hereunto set my hand this 31st day of January, 1906.

LAWRENCE E. BARRINGER.

Witnesses:

BENJAMIN B. HULL,  
HELEN ORFORD.